

Patented Dec. 8, 1925.

1,564,414

# UNITED STATES PATENT OFFICE.

CLAYTON M. HOFF, OF CLEVELAND, OHIO. ASSIGNOR TO THE GRASSELLI CHEMICAL COMPANY, OF CLEVELAND, OHIO, A CORPORATION OF OHIO.

## CADMIUM PLATING.

No Drawing.

Application filed October 6, 1924. Serial No. 742,073.

To all whom it may concern:

Be it known that I, CLAYTON M. HOFF, a citizen of the United States, residing at Cleveland, in the county of Cuyahoga and 5 State of Ohio, have invented certain new and useful Improvements in Cadmium Plating, of which the following is a specification.

This invention relates to the electroplating of cadmium and more particularly to a 10 composition for that purpose.

In my application Serial No. 686,898, filed Jan. 17, 1924. I have disclosed a process of electroplating cadmium involving the use of an alkaline bath containing chemical 15 combinations of cyanide, ammonium and cadmium, with or without addition agents such as gulac which may be prepared for instance by dissolving cadmium oxid or hydroxid or a salt such as cadmium sulfate in aqua- 20 ammonia and adding thereto a soluble cyanide such as sodium cyanide.

Such a bath is characterized by the fact that from it pure, smooth and uniform deposits of cadmium may be produced rapidly 25 and quantitatively if desired, even when the bath contains other metals such as zinc.

It is desirable for the chemicals manufacturer to be able to supply the electroplater with the materials required ready for use, 30 but since it is not feasible to ship and store the finished electroplating bath, it is customary when possible to supply the electroplater with a mixture of chemicals ready to be dissolved in water to produce the bath.

It is therefore an object of my present invention to provide a dry mixture of chemicals suitable for storage and shipment which when dissolved in water, with or without other materials as will appear hereinafter, 35 will give a cadmium plating bath having in general the characteristics of the bath disclosed in my application above referred to. In the course of my investigations in this connection for the purpose of developing such a dry mixture of chemicals I have 40 found that baths having the desired characteristics may be prepared in a variety of ways.

As stated above the bath of my earlier 45 application comprises as essential ingredients or components cadmium, ammonium, cyanide and an alkaline agent. Each of these components may be supplied in various forms. For instance the cadmium component may be supplied in the form of the

oxid, hydroxid, or cyanide, or in the form of a salt such as the sulfate. The cyanide component may be supplied in chemical combination with the cadmium as cadmium cyanide or as ammonium cyanide, or as other metal cyanides, preferably those of the alkali metals. The ammonium component may be supplied in the form of ammonium hydroxide or as a salt such as ammonium cyanide or sulfate. The ammonium component apparently serves as the agent which prevents or tends to prevent the deposition of other metals, particularly zinc, along with the cadmium and may be replaced by other materials such as sodium sulfate 60 and other alkali metal salts. The alkaline reaction of the bath may be produced by the use of ammonia or an alkali metal hydroxid. The bath preferably is made to contain also a colloid agent, which tends to 65 improve the quality of the cadmium plate, such as starch, gulac, dextrine, etc.

The following examples of bath compositions illustrate my invention:

### Example 1.

3 oz., cadmium hydroxide; 6½ to 7 oz., sodium cyanide; ½ to 1 oz., caustic soda; ¼ to ½ oz., sodium carbonate, and 1 oz., 70 aqua ammonia 26° Bé. to each gallon of water.

### Example 2.

40 oz., cadmium hydroxide; 30 oz., ammonium sulfate; 85 oz., sodium cyanide; 13 oz., sodium hydroxide, and 9 oz., gulac to 75 each 5 gallons of water.

From the foregoing description it is apparent that compositions having the characteristics of those illustrated in the foregoing examples, that is, being alkaline and containing cadmium, cyanide, ammonium or another agent which tends to prevent the co-deposition of other metals such as zinc with or without an addition agent such as gulac may be produced in a great variety of ways, that is by the use of a great variety of chemicals. The relative proportions of the ingredients and the concentration of the bath may 80 of course be varied without departing from my invention.

Of the great variety of combinations of chemicals indicated above only a comparatively few are well adapted from an 85

economical and practical standpoint for commercial use. A dry mixture suitable for shipment may be composed of for example cadmium hydroxide, ammonium sulfate, sodium cyanide, sodium hydroxide and gulac, or since the shipment of caustic soda and cyanide is somewhat objectionable, the electroplater may be supplied with a mixture of cadmium hydroxide, ammonium sulfate and 5 gulac with directions as to the quantity thereof to be dissolved in a given quantity of water along with caustic soda and sodium cyanide separately supplied. Or the electroplater may be supplied with a dry mixture 10 of cadmium hydroxide, sodium hydroxide, sodium cyanide and gulac, to which ammonia or an ammonium salt is to be added 15 in the preparation of the bath. These few examples as given are sufficient for the purposes of illustration, it being understood 20 that the invention is not limited to the particular combinations of chemicals instanced. The electroplating from baths comprising the combinations of chemicals described may 25 be carried out as disclosed in my prior application, for instance at room temperature using a potential of 4 to 6 volts and a current density of 1 ampere per 100 square centimeters between electrodes spaced about 30 15 centimeters apart, and preferably using cadmium anodes with an anode surface area equal to two or three times the cathode surface area. Known expedients such as agitation or circulation or heating or cooling of 35 the bath, rotation of the electrodes, etc., may be employed.

I claim:

1. A composition adapted for use in the electrodeposition of cadmium comprising a 40 cadmium compound, a material which tends to prevent the co-plating of zinc with cadmium, an alkaline agent, a cyanide, and a material which tends to improve the quality of cadmium platings.
2. A composition adapted for use in the 45 electrodeposition of cadmium comprising a cadmium compound, a material which tends to prevent the co-plating of zinc with cadmium, an alkaline agent and a cyanide.

3. A composition adapted for use in the 50 electrodeposition of cadmium comprising a cadmium compound, an ammonium compound, an alkaline agent and a cyanide.

4. A composition adapted for use in the 55 electrodeposition of cadmium comprising a cadmium compound, an ammonium compound, a caustic alkali, and an alkali metal cyanide.

5. A composition adapted for use in the 60 electrodeposition of cadmium comprising a cadmium hydroxide, an ammonium compound, an alkaline agent and a cyanide.

6. A composition adapted for use in the 65 electrodeposition of cadmium comprising a cadmium hydroxide, ammonium sulfate, an alkali metal hydroxide and an alkali metal cyanide.

7. A composition of matter adapted for 70 use for the preparation of a cadmium plating bath consisting of a dry mixture comprising a cadmium compound and a material which tends to prevent the co-plating of zinc.

8. A composition of matter adapted for 75 use for the preparation of a cadmium plating bath consisting of a dry mixture comprising a cadmium compound and an ammonium salt.

9. A composition of matter adapted for 80 use for the preparation of a cadmium plating bath consisting of a dry mixture comprising cadmium hydroxide and ammonium sulfate.

10. A composition of matter adapted for 85 use for the preparation of a cadmium plating bath consisting of a dry mixture comprising a cadmium compound, a material which tends to prevent the co-plating of zinc, and a material which tends to improve the quality of cadmium platings.

11. A composition of matter adapted for 90 use for the preparation of a cadmium plating bath consisting of a dry mixture comprising a cadmium compound, an ammonium salt and an addition agent.

12. A dry mixture of cadmium hydrate, 95 ammonium sulfate and gulac.

In testimony whereof, I affix my signature.

CLAYTON M. HOFF.